

1

3,276,979

**BATHS AND PROCESSES FOR THE PRODUCTION  
OF METAL ELECTROPLATES**

Wennemar Strauss and Wolf-Dieter Willmund, Dusseldorf-Holthausen, Germany, assignors to Dehydag Deutsche Hydrierwerke G.m.b.H., Dusseldorf, Germany, a corporation of Germany

No Drawing. Filed Aug. 23, 1962, Ser. No. 218,841  
Claims priority, application Germany, Aug. 31, 1961,

D 36,927

18 Claims. (Cl. 204—49)

This invention relates to improved brightening additives for electroplating baths and to the electroplating process using these brighteners. It more particularly relates to the use of organic sulfonic acid derivatives in electroplating baths whereby the electroplating process may be operated at higher temperatures.

It is known from German Patent No. 888,493 that electrolyte soluble derivatives of esters of sulfothio or trithiocarbonic acid or of dithiocarbamic acid, which contain the grouping



at least once in the molecule, can be added to copper electroplating baths of customary compositions in order to achieve an improved brightening effect on the objects to be copper electroplated. The solubilizing group, a carboxyl or sulfonic acid group, in these derivatives is attached to the sulfur atom of the



grouping through a short chain bivalent aliphatic radical. At bath temperatures up to about 30° C., these additives exhibit an excellent brightening effect, but their leveling effect is not always completely satisfactory.

It is an object of this invention to provide an electroplating bath and process for obtaining bright and level electrodeposits of metals.

A further object of this invention is to provide an electroplating process and bath operable at higher temperatures.

Another object is to provide additives for electroplating baths which give both a brightening and a leveling effect.

These and other objects of my invention will become apparent as the description thereof proceeds.

We have now found that it is possible to obtain full bright electrodeposits of copper, nickel, zinc, cadmium, and other metals with good leveling properties at even still higher temperatures up to about 50° C. when the baths of customary compositions are modified with those sulfonic acids or their salts which contain one or more carbon atoms which are attached only to heteroatoms and in which the sulfonic acid group is attached to the sulfur atom of a



grouping through a bivalent hydrocarbon radical which contains an aryl group. Compounds of the type contemplated in accordance with the invention are characterized by the following general formula:



In this formula R represents an aliphatic, cycloaliphatic or aromatic hydrocarbon radical, X is a heteroatom such as oxygen, NR" (R"=H or R) or S, R' is a bivalent hydrocarbon radical, which contains an aryl group, and G is a cation of an inorganic or organic base or also

2

hydrogen. In the event that R" represents an aliphatic radical, the substituents R and R" may also form a ring system together with the nitrogen atom, which may contain a further heteroatom.

Compounds of this type are obtained in known fashion, for example, by reaction of dithiocarbamates with tolylsultone (inner ester of O-oxymethyl sulfonic acid), correspondingly substituted tolyl sulfones or halogenalkylsulfonates. The latter are accessible through halogenation of alkylsulfonates, for instances, in suspension in a high-boiling point inert solvent which is inert toward halogen or by treatment of the halogen alkyl aromates with chlorosulfonic acids at -20° C. or with thionyl chloride; in the last case a hydrolysis of the sulfonylchloride to form sulfonic acid must be excluded. The following are a few examples of salts of such aromatic sulfonic acids which contain alkyl radicals and which may be used as bright electroplating additives in accordance with the present invention:

- 20 N,N-diethyl-dithiocarbamic acid S-benzylerster-o-sodium sulfonate,  
N-butyl-dithiocarbamic acid-S-benzylerster-p-sodium sulfonate,  
25 S-phenyl-trithiocarbonate acid-S-benzylerster-o-sodium sulfonate,  
N,N-1,5-pentamethylene-dithiocarbamic acid-S-  
benzylerster-o-sodium sulfonate,  
N,N-1,5-pentamethylene-dithiocarbamic acid-S-(m-  
30 methyl)-benzylerster-sodium sulfonate,  
3-oxa-N,N-1,5-pentamethylene-dithiocarbamic acid-S-  
(p-methyl)-2-phenylethylester-sodium sulfonate,  
S-phenyl-trithiocarbonic acid-S-(3,5-dimethyl)-benzylerster sodium sulfonate,  
35 n-Butyl-xanthogenic acid-S-naphthyl-methyl ester  
sodium sulfonate,

the reaction product of diethyl dithio carbamate and tetrapropylene benzene sodium sulfonate which is halogenated in the carbon chain, and the like.

40 The electroplating additives according to the present invention may be employed in all types of electroplating processes, especially for copper plating, nickel plating, silver plating, zinc plating, as well as for the preparation of cadmium, bronze or brass electroplates. These agents 45 may also be employed in conjunction with other known brightening agents as well as with leveling agents, porosity prevention agents, hardness binding agents, inhibitors, wetting agents, conductive salts, etc.

50 The amounts in which the agents according to the present invention, are added to the baths lie between about 0.01 to 20 g./l. of bath fluid. In general, the baths are operated at current densities between 0.5 and 12 amperes per dm.<sup>2</sup>, and in special cases at temperatures up to 70° C. It should be particularly emphasized that in 55 the case of an acid copper electroplating bath, the bath containing the agents according to the present invention may be operated within a temperature range of 15 to 50° C., and under these conditions the bath produces complete mirror brightening effects and the leveling effect of the baths as a rule completely satisfies the practical requirements.

60 The base metal to be electroplated may be any type of metal previously employed for this purpose, such as iron, steel, zinc, and other non-precious metals or metal alloys. If necessary, in conjunction with the copper electroplating of non-precious metals, the base metal is as usual provided with a thin preliminary copper plate in a cyanide bath. However, the baths according to the 65 present invention may also be employed with success in the direct acid copper plating process, that is, by subjecting the objects to be copperplated to a preliminary



ing 220 g./l. of copper sulfate and 60 g./l. of sulfuric acid. The bright copper electroplates obtained with the aid of this bath extend at room temperature from about 0.5 to 8 amperes per dm.<sup>2</sup>. The addition of a wetting agent is not required.

While we have set forth certain specific embodiments and preferred modes of practice of our invention, it will be understood that the invention is not limited thereby, and that various changes and modifications may be made without departing from the spirit of the disclosure or the scope of the appended claims.

We claim:

1. An electroplating bath for producing bright and level electrodeposits of metals selected from the group consisting of copper, nickel and zinc comprising an acid aqueous solution of the metal to be electrodeposited and an additive compound of the formula



wherein R is selected from the group consisting of aliphatic, cycloaliphatic and aromatic radicals, X is selected from the group consisting of —O—, —S— and —NR''—, R'' is selected from the group consisting of hydrogen and aliphatic, cycloaliphatic and aromatic radicals and R and R'' taken together with the nitrogen atom may form a heterocyclic radical, R' is a bivalent hydrocarbon radical having an aryl group to which the —SO<sub>3</sub>G group is attached and G is selected from the group consisting of hydrogen and alkali metal; said additive being added in sufficient amount to obtain said bright and level electrodeposit.

2. An electroplating bath for producing bright and level electrodeposits of metals selected from the group consisting of copper, nickel and zinc comprising an acid aqueous solution of the metal to be electrodeposited and from 0.01 to 20 g./l. of an additive compound of the formula



wherein R is selected from the group consisting of aliphatic, cycloaliphatic and aromatic radicals, X is selected from the group consisting of —O—, —S— and —NR''—, R' is selected from the group consisting of hydrogen and aliphatic, cycloaliphatic and aromatic radicals and R and R'' taken together with the nitrogen atom may form a heterocyclic radical, R' is a bivalent hydrocarbon radical having an aryl group to which the —SO<sub>3</sub>G group is attached and G is selected from the group consisting of hydrogen and alkali metal.

3. An electroplating process for producing bright and level electrodeposits of metals selected from the group consisting of copper, nickel and zinc comprising electrodepositing the said metals from a bath comprising an acid aqueous solution of the metal to be electrodeposited in the presence of an additive compound of the formula



wherein R is selected from the group consisting of aliphatic, cycloaliphatic and aromatic radicals, X is selected from the group consisting of —O—, —S— and —NR''—, R'' is selected from the group consisting of hydrogen and aliphatic, cycloaliphatic and aromatic radicals and R and R'' taken together with the nitrogen atom may form a heterocyclic radical, R' is a bivalent hydrocarbon radical having an aryl group to which the —SO<sub>3</sub>G group is attached and G is selected from the group consisting of hydrogen and alkali metal.

4. An electroplating process for producing bright and level electrodeposits of metals selected from the group consisting of copper, nickel and zinc, comprising electrodepositing the said metals from a bath comprising an acid aqueous solution of the metal to be electrodeposited

in the presence of from 0.01 to 20 g./l. of an additive compound of the formula



wherein R is selected from the group consisting of aliphatic, cycloaliphatic and aromatic radicals, X is selected from the group consisting of —O—, —S— and —NR''—, R'' is selected from the group consisting of hydrogen and aliphatic, cycloaliphatic and aromatic radicals and R and R'' taken together with the nitrogen atom may form a heterocyclic radical, R' is a bivalent hydrocarbon radical having an aryl group to which the —SO<sub>3</sub>G group is attached and G is selected from the group consisting of hydrogen and alkali metal.

5. An electroplating bath for producing bright and level electrodeposits of metals selected from the group consisting of copper, nickel and zinc comprising an acid aqueous solution of the metal to be electrodeposited and from 0.01 to 20 g./l. of an additive compound having a structural formula as follows:



6. An electroplating bath for producing bright and level electrodeposits of metals selected from the group consisting of copper, nickel, and zinc comprising an acid aqueous solution of the metal to be electrodeposited and from 0.01 to 20 g./l. of an additive compound having a structural formula as follows:



7. An electroplating bath for producing bright and level electrodeposits of metals selected from the group consisting of copper, nickel, and zinc comprising an acid aqueous solution of the metal to be electrodeposited and from 0.01 to 20 g./l. of an additive compound having a structural formula as follows:



8. An electroplating bath for producing bright and level electrodeposits of metals selected from the group consisting of copper, nickel, and zinc comprising an acid aqueous solution of the metal to be electrodeposited and from 0.01 to 20 g./l. of an additive compound having a structural formula as follows:



9. An electroplating bath for producing bright and level electrodeposits of metals selected from the group consisting of copper, nickel, and zinc comprising an acid aqueous solution of the metal to be electrodeposited and from 0.01 to 20 g./l. of an additive compound having a structural formula as follows:



10. An electroplating bath for producing bright and level electrodeposits of metals selected from the group consisting of copper, nickel, and zinc comprising an acid aqueous solution of the metal to be electrodeposited

and from 0.01 to 20 g./l. of an additive compound having a structural formula as follows:



11. An electroplating bath for producing bright and level electrodeposits of metals selected from the group consisting of copper, nickel, and zinc comprising an acid aqueous solution of the metal to be electrodeposited and from 0.01 to 20 g./l. of an additive compound having a structural formula as follows:



12. An electroplating process for producing bright and level electrodeposits of metals selected from the group consisting of copper, nickel, and zinc comprising electrodepositing the metals from a bath comprising an acid aqueous solution of the metal to be electrodeposited and from 0.01 to 20 g./l. of an additive compound having a structural formula as follows:



13. An electroplating process for producing bright and level electrodeposits of metals selected from the group consisting of copper, nickel, and zinc comprising electrodepositing the metals from a bath comprising an acid aqueous solution of the metal to be electrodeposited in the presence of from 0.01 to 20 g./l. of an additive compound having a structural formula as follows:



14. An electroplating process for producing bright and level electrodeposits of metals selected from the group consisting of copper, nickel, and zinc comprising electrodepositing the metals from a bath comprising an acid aqueous solution of the metal to be electrodeposited in the presence of from 0.01 to 20 g./l. of an additive compound having a structural formula as follows:



15. An electroplating process for producing bright and level electrodeposits of metals selected from the group consisting of copper, nickel, and zinc comprising electrodepositing the metals from a bath comprising an acid aqueous solution of the metal to be electrodeposited in

8  
the presence of from 0.01 to 20 g./l. of an additive compound having a structural formula as follows:



16. An electroplating process for producing bright and level electrodeposits of metals selected from the group consisting of copper, nickel, and zinc comprising electrodepositing the metals from a bath comprising an acid in the presence from 0.01 to 20 g./l. of an additive compound having a structural formula as follows:



17. An electroplating process for producing bright and level electrodeposits of metals selected from the group consisting of copper, nickel, and zinc comprising electrodepositing the metals from a bath comprising an acid aqueous solution of the metal to be electrodeposited in the presence of from 0.01 to 20 g./l. of an additive compound having a structural formula as follows:



18. An electroplating process for producing bright and level electrodeposits of metals selected from the group consisting of copper, nickel, and zinc comprising electrodepositing the metals from a bath comprising an acid aqueous solution of the metal to be electrodeposited in the presence of from 0.01 to 20 g./l. of an additive compound having a structural formula as follows:



#### References Cited by the Examiner

##### UNITED STATES PATENTS

|           |        |                |     |    |
|-----------|--------|----------------|-----|----|
| 2,830,014 | 4/1958 | Gundel et al.  | 204 | 49 |
| 2,837,472 | 6/1958 | Gundel et al.  | 204 | 49 |
| 2,849,351 | 8/1958 | Gundel et al.  | 204 | 44 |
| 2,937,978 | 5/1960 | Strauss et al. | 204 | 49 |

##### FOREIGN PATENTS

|         |         |                |  |
|---------|---------|----------------|--|
| 572,016 | 10/1958 | Belgium.       |  |
| 572,186 | 11/1958 | Belgium.       |  |
| 888,493 | 9/1953  | Germany.       |  |
| 873,753 | 7/1961  | Great Britain. |  |

JOHN H. MACK, Primary Examiner.

G. KAPLAN, Assistant Examiner.